

June 22, 1926.

1,590,034

F. C. KELLEY

METAL COATING

Filed May 10, 1920



Inventor:  
Floyd C. Kelley,  
by *Arthur L. Davis*  
His Attorney.

## UNITED STATES PATENT OFFICE.

FLOYD C. KELLEY, OF SCHENECTADY, NEW YORK, ASSIGNOR TO GENERAL ELECTRIC COMPANY, A CORPORATION OF NEW YORK.

## METAL COATING.

Application filed May 10, 1920. Serial No. 380,023.

The present invention relates to the coating of cast iron with other metal and particularly to the production of a composite article of cast iron and a nonferrous metal. Great difficulty has been experienced in causing cast iron to unite with a non-ferrous metal, for example, copper, in such a way as to produce a thoroughly adherent coating or union. Heating the metals to be united in hydrogen does not cause the copper to wet the cast iron as is the case when copper in a molten state is brought into contact with steel in the presence of hydrogen. Fluxes likewise fail to produce an adherent coating between cast iron and copper, or the like, when used in the usual way in contact with air.

I have discovered that a homogeneously adherent union between cast iron and a non-ferrous metal of lower melting point, such as copper, silver or brass can be produced by applying the molten non-ferrous metal to the cast iron to be coated in a reducing atmosphere in the presence of a flux, particularly cryolite.

In accordance with my invention, cast iron articles intimately united with brass or other suitable cupreous metal, may be produced. The cupreous metal in turn may be united with a layer of other metal, such for example, as Babbitt metal which otherwise could not be integrally united with cast iron.

The accompanying drawing illustrates in section a bearing made by the practice of a process embodying my invention.

In accordance with one method of carrying out my invention a body of cast iron 1 to be joined to a metal layer 2 of copper, silver or the like is heated in any convenient way, as for example, in an ordinary gas flame, to about 750 to 800° C., whereby the surface of the cast iron is oxidized. A suitable flux, preferably cryolite, then is distributed uniformly over the heated surface as by applying the cryolite in powdered form upon the oxidized surface of the cast iron. The cryolite is brought to fusion on the heated cast iron, and the iron surface coated with cryolite flux is brought into contact with molten copper, brass or the like in a hydrogen atmosphere. For example, a

piece of copper wire may be wrapped about the cast iron and the iron with the copper heated to the melting point of copper in a hydrogen furnace. If the cryolite has been properly distributed before melting the copper, a uniform coating 2, of copper results which when molten "wets" the cast iron in such a way as to resist mechanical separation when solidified. The heating of the cast iron to a temperature of about 750° to 800° C. in an ordinary gas flame decarburizes the surface of the cast iron or, in other words, oxidizes the carbon out of the surfaces of the cast iron, and whatever oxide of the iron is formed is subsequently reduced by the hydrogen.

A layer of Babbitt metal 3 may be cast against the layer of copper. A bearing thus produced may be supported on a suitable frame 4. Only one-half of the bearing enclosing the shaft 5 has been illustrated.

When cast iron is to be coated with silver, I prefer to employ borax as a flux.

In the appended claims, I have set forth the novel features of my invention with particular reference to copper but I wish it to be understood that my invention is equally applicable to coating cast iron with other metals, as for example, brass.

What I claim as new and desire to secure by Letters Patent of the United States, is:—

1. The method of coating cast iron with a non-ferrous metal which comprises heating the cast iron to a temperature sufficiently high to decarburize the surface to be coated, applying cryolite to said surface and bringing copper in a molten state into contact with the cryolite coated surface in a reducing atmosphere.

2. The method of coating cast iron with copper which consists in heating cast iron to a temperature of about 750° C. to 800° C. in a gas flame, coating the heated surface of said iron with cryolite, and thereupon bringing melted copper into contact with said surface in a hydrogen atmosphere.

3. The method of coating cast iron with a non-ferrous metal of lower melting point than cast iron which consists in heating the cast iron to about 750 to 800° C. in an oxidizing flame and thereupon applying

said non-ferrous metal to the oxidized surface in the presence of both a flux and a reducing gas.

4. The method of producing an adher-  
5 ent coating of copper upon cast iron which comprises first heating the cast iron in an open flame to thereby decarburize the sur-

face of the cast iron, applying a flux upon said surface, fusing said flux and applying copper in a fused state and in a hydrogen 10 atmosphere to the flux coated surface.

In witness whereof, I have hereunto set my hand this 7th day of May, 1920.

FLOYD C. KELLEY.